

## 1

3,079,220

INHIBITING CORROSION WITH CHROMIUM-  
QUATERNARY AMMONIUM SALT COMPO-  
SITIONS

David B. Boies, Chicago, Jean Crowther, Evanston, and  
Walter J. Ryzner, Chicago, Ill., assignors to Nalco  
Chemical Company, Chicago, Ill., a corporation of  
Delaware  
No Drawing. Filed Sept. 10, 1959, Ser. No. 839,077  
22 Claims. (Cl. 21—2.7)

This invention relates to a new method for inhibiting corrosion in industrial process water systems. More specifically, it relates to non-corrosive aqueous liquids which contain minor amounts of corrosion inhibiting chemicals.

In under water systems in which water moves through such units as condensers, engine jackets, cooling towers and the like, corrosion is frequently quite severe due to the fact that water is concentrated several times during the course of the various processes. Such systems which are for the most part, recirculating types, contain equipment which uses as its structural material such metals as iron and steel, brass, copper, admiralty metal as well as minor amounts of zinc and other non-ferrous metals.

One of the best inhibitors for rendering such systems non-corrosive are the well known alkali metal chromates. While chromates are economical and give good results, in many cases it has frequently been the experience of the art that pitting and tuberculation of the various surfaces occurs when chromates are used alone. The problem of pitting and tuberculation which sometimes occurs with chromate inhibitors may be mitigated using chromates in conjunction with phosphates. Although such combinations of inhibitors have proven to be of value in protecting industrial process water systems, they are not entirely satisfactory from all standpoints.

Many attempts have been made to develop new inhibitors for aqueous systems of the type described above, with much effort being directed towards discovering an organic inhibitor of the so-called film forming type. Materials such as amine compounds, quaternary ammonium salts, and certain carboxylic acids which are known to be effective inhibitors for many types of systems have failed to protect industrial process water systems at low economical dosages.

It would be a valuable contribution to the art if an inhibitor containing an organic film forming component could be devised for industrial process systems which would be effective at low economical dosages and would be successful in preventing tuberculation and pitting of metals in contact with such systems.

It has been discovered that extremely valuable corrosion protection to metals in contact with industrial process waters may be afforded by treating such systems with a combination treatment which comprises a water soluble hexavalent chromium compound in conjunction with a specific type of water dispersible quaternary ammonium salt. In a preferred embodiment, the water soluble hexavalent chromium compounds and the water dispersible quaternary ammonium salts are advantageously combined with minor amounts of certain compounds capable of producing in aqueous solution a heavy metal cation such as zinc, cobalt, nickel, mercury and trivalent chromium cations.

The various compositions described above as the inhibitors of the invention are preferably used at certain

## 2

dosage levels in the water to provide optimum results. In the case of the hexavalent chromium compounds, the dosage is maintained at between 10 and 200 parts per million (expressed as  $\text{CrO}_4$ ). Preferably the dosage is maintained between 15 and 50 parts per million. The quaternary ammonium salt is maintained in the water at a dosage level ranging at generally between 0.5 to 10 parts per million and preferably between 2 and 6 parts per million. In the case of the heavy metal compounds, the dosage is maintained at between 0.25 and 10 parts per million with the preferred range being at 2 to 6 parts per million. These latter dosages are expressed in terms of the metal rather than the total compound with which it is associated.

15 In order to achieve optimum results, it is beneficial that the pH of the water be maintained within certain specific ranges. As a general rule, these ranges may vary between 5.5 and 8.5, although the best results are achieved when the pH is kept within the ranges of 6.5 to 7.5.

20 The hexavalent compounds of chromium are most suitably chosen from the alkali metal chromates and dichromates such as sodium dichromate dihydrate, sodium chromate (anhydrous), sodium chromate tetrahydrate, sodium chromate hexahydrate, sodium chromate decahydrate, potassium dichromate, potassium chromate, and the like.

25 The quaternary ammonium salts used in the practice of the invention may be selected from a large group of known and commercially available materials. It is essential to the practice of the invention that the particular quaternary ammonium salt must contain at least 8 carbon atoms and preferably at least one acyclic organic radical of at least 12 carbon atoms in chain length. The higher acyclic organic radical may contain as many as 22 carbon atoms. Preferably the higher acyclic organic radical should be from 16 to 18 carbon atoms in chain length. A preferred group of quaternary ammonium salts are the quaternary ammonium chlorides having the following general structural formulae:



30 where R is a higher aliphatic group of from 16-18 carbon atoms in chain length, e.g., hexadecyl, heptadecenyl, octadecyl, and octadecenyl, and  $\text{R}_1$ ,  $\text{R}_2$  and  $\text{R}_3$  are lower aliphatic carbon groups of from 1-6 carbon atoms in chain length, e.g., methyl, ethyl, propyl, isopropyl, butyl, isobutyl, amyl, isoamyl, and hexyl. Another useful group of quaternary ammonium salts are the higher aliphatic substituted imidazolinium salts.

35 For purposes of illustrating several quaternary ammonium salts of the type which may be used in the practice of the invention, Table I is presented. Also included in this table are certain amines which are considered inoperative.

TABLE I

*Quaternary Ammonium Salts*

- 40 A. Imidazolinium salts:
- (1) 2-methyl-1-(2-hydroxy ethyl)-1-benzyl imidazolinium chloride
  - (2) 2-coco-1-(2-hydroxyethyl)-1-benzyl imidazolinium chloride
  - (3) 2-coco-1-(hydroxyethyl)-1-(4-chlorobutyl imidazolinium chloride

- (4) 2-coco-1-(2-hydroxyethyl)-1-octadecenyl imidazolinium chloride
- (5) 2-tall oil fatty-1-(2-hydroxyethyl)-1-benzyl imidazolinium chloride<sup>1</sup>
- (6) 2-tall oil fatty-1-(2-hydroxyethyl)-1-(4-chlorobutyl) imidazolinium chloride<sup>1</sup>
- (7) 2-heptadecenyl-1-(2-hydroxyethyl)-1-(4-chlorobutyl) imidazolinium chloride
- (8) 2-heptadecenyl-1-(2-hydroxyethyl)-1-benzyl imidazolinium chloride
- (9) 2-heptadecyl-1-(hydroxyethyl)-1-octadecyl imidazolinium ethyl sulfate

B. Aliphatic quaternaries:

- (10) Dodecyl trimethyl ammonium chloride
- (11) Hexadecyl trimethyl ammonium chloride
- (12) Octadecyl trimethyl ammonium chloride
- (13) Coco trimethyl ammonium chloride
- (14) Soya trimethyl ammonium chloride
- (15) Tallow trimethyl ammonium chloride
- (16) Dicoco dimethyl ammonium chloride
- (17) Coco amine Rx 15 moles EtO quaternized with methyl chloride
- (18) Octadecyl amine Rx 2 moles EtO quaternized with methyl chloride
- (19) Octadecenyl amine Rx 2 moles EtO quaternized with methyl chloride
- (19A) Di(hydrogenated tallow) dimethyl ammonium chloride

C. Amines:

- (20) Soya amine
- (21) Hydrogenated tallow amine
- (22) Coco amine

D. Miscellaneous quaternary ammonium compounds:

- (23) Lauryl isoquinolinium bromide
- (24) Cetyl isoquinolinium bromide
- (25) Lauryl isoquinolinium chloride
- (26) Alkyl (C<sub>8</sub>H<sub>17</sub> to C<sub>18</sub>H<sub>37</sub>) dimethyl-3,4-dichlorobenzyl ammonium chloride and alkenyl (C<sub>16</sub> to C<sub>20</sub>) dimethyl ethyl ammonium bromides in the ratio 5:1
- (27) Octadecenyl-9-dimethyl benzyl ammonium chloride
- (28) 1-dodecyl-2-benzyl pyridinium bromide
- (29) 1-methyl-2-ethyl piperidinium bromide
- (30) Hexadecyl pyridinium bromide
- (31) N-soya-N ethyl morpholinium ethosulfate

From the above table it will be seen that the quaternary ammonium salt may have a wide variety of substituents just so long as they contain a higher aliphatic group of the type previously specified. Other useful imidazolinium salts which meet the specifications set forth herein are disclosed in Rydell, U.S. 2,738,325. The preferred quaternary ammonium salts have only one higher saturated or unsaturated aliphatic group of at least 12 carbon atoms since they are most readily dispersible in the aqueous systems in which they are employed. The higher aliphatic radicals may be mixed, as, for example, those radicals derived from vegetable oils and animal fats. The expression "dispersible" when referring to the quaternary ammonium salts is meant to refer to those materials that are either water soluble or those that may be colloidally dispersed in aqueous systems at use concentrations.

The heavy metal cations are derived from their water soluble salts or bases. Examples of typical compounds that fall within this category are the following: zinc sulfate, cobaltous chloride, nickel iodide, mercuric acetate, chromic chloride, zinc chloride, cobaltous sulfate, and mercurous chloride.

When making concentrated solutions for the purpose of feeding, it is frequently desirable to use the acidic salts of the heavy metal materials such as, for instance, zinc sulfate and also to use an acid or an acidic material

such as sodium hydrogen sulfate or sulfamic acid whereby the pH of the resulting concentrated solution is adjusted between 3.5 and 5.

In using the inhibitors described above, it is helpful if the hexavalent chromium compounds and the heavy metal ionizable compound is combined into one formulation. The quaternary ammonium salt is used as a separate entity, since experience has shown that combining all the ingredients into a unitary product causes a reaction to occur between the chromate and the quaternary ammonium salt, which reaction forms an insoluble material. When fed separately to industrial process water systems at the dosages previously specified, no such insoluble reaction products are formed. Typical products of the invention have the following formulae:

|    | A                    |      |
|----|----------------------|------|
|    | Sodium dichromate    | 65.7 |
|    | Sodium polyphosphate | 3.7  |
| 20 | Zinc sulfate         | 28.5 |
|    | Sodium bisulfate     | 1.0  |
|    | Water                | 1.1  |

|  | B                                     |      |
|--|---------------------------------------|------|
|  | Octadecyl trimethyl ammonium chloride | 25.0 |
|  | Isopropanol                           | 40.0 |
|  | Water                                 | 35.0 |

The polyphosphate in Formula A is added for the purpose of stabilizing the calcium carbonate which may be present in the water. If calcium carbonate does not present a problem in the water to be treated, the polyphosphate is omitted. However, since this process does not adversely affect the usefulness of the treatments, it is desirable to use it in most cases. The phosphate may be used in dosages of .5 to 2 parts per million, although dosages as high as 1 to 9 parts per million may also be used, but generally the dosage need never exceed 1 part per million. It should be noted that at these dosage levels the phosphate neither adds nor detracts from the inhibiting properties of the compositions described above.

EVALUATION OF THE INVENTION

The test methods used to determine the efficacy of the invention when used to inhibit the corrosion of industrial process waters are of three types. These test methods are described below in detail under the headings of test methods A, B, and C.

*Test method A.*—The specimens used are weighed, sandblasted mild steel coupons (SAE 1010) 1 inch wide by 2 inches long by 20 gauge. 500 ml. of the test water was used. The treatment was added (generally from a stock solution) and the pH adjusted to 6.5 with sulfuric acid or sodium hydroxide. The test water was prepared to simulate a typical cooling water. This synthetic water had the following composition:

|                                               | P.p.m. |
|-----------------------------------------------|--------|
| Total hardness (as CaCO <sub>3</sub> )        | 400    |
| Calcium hardness (as CaCO <sub>3</sub> )      | 250    |
| Magnesium hardness (as CaCO <sub>3</sub> )    | 150    |
| 60 Total alkalinity (as CaCO <sub>3</sub> )   | 5      |
| Sulfate (as Na <sub>2</sub> SO <sub>4</sub> ) | 1400   |
| Chloride (as NaCl)                            | 500    |

The test coupon was immersed and the solution stirred at 1750 r.p.m. with a bell shaped stirrer for 24 hours. At the end of this time the coupon was removed from the water and air dried. The coupon was then examined and scored according to the weight loss of the coupon and visual evaluation of factors such as pitting and deposit.

70 The test was run at 140° F.

*Test method B.*—The second laboratory testing procedure was also quantitative in nature and involved measurement of corrosion rates of metallic coupons. These were subjected to certain specific sets of test conditions designed to approximate those found in field

<sup>1</sup> Essentially free from rosin acid components.

operation which contribute to the corrosion. While it was obviously necessary to make some adjustments for small scale laboratory testing, a strong effort was made to incorporate those variables which are the major factors in causing corrosion in heat exchangers associated with cooling tower systems. The principal corrosive factors operating on the coupons are:

High dissolved oxygen level  
High chlorides, sulfates and total dissolved solids  
Low alkalinity, low pH (6-6.5)

This test combined the advantages of both the "batch" type test and the "once through" test and was essentially an intermittent, once-through test. With this system, conditions were maintained constant throughout the test while a relatively small volume of water was used.

The equipment consisted of a series of individual units. Each unit was complete and independent of the others. It consisted of a five-gallon bottle which formed the reservoir for the test water. The water flowed from the reservoir by gravity to a feed assembly that controlled the head level. From there the water passed through a solenoid valve that was activated by an electrical timer. The timer opened the valve every eighteen minutes to allow 40 ml. of the water to flow into the test vessel that was partially immersed in a constant-temperature oil bath at 140° F. The rate of flow was about 3.2 liters per day, corresponding to a 1.3 fold replacement of the water daily. The water left the test vessel through an overflow tube. The standard water used in this test had the same composition as the one used in Test Method A. Variations covering a range of typical cooling waters have been checked with results similar to those described here.

The test specimens were made of No. 20 gauge SAE 1010 mild steel, and were one inch wide and 2 inches long. They were suspended in the test vessel from a  $\frac{3}{16}$  inch hole drilled  $\frac{1}{4}$  inch for the short edge. The panels were prepared by sandblasting with "flint shot" sand. After sandblasting they were cleaned first in toluene and then in acetone, and weighed and placed in the test vessel. After the test they were removed and then cleaned by a 30 second immersion in muriatic acid inhibited with formaldehyde. They were then removed from the acid and neutralized in a soda ash solution. The panels were then rinsed in water, dipped in acetone and air dried. Test panels were stored in a heated cabinet at 105° F. before weighing.

The test vessel was a Pyrex jar 6 inches in diameter and 8 inches tall, with an overflow tube at a point two inches from the top. The vessel was covered by a stainless steel lid that had a hole in the center to accommodate the stirrer, and holes around the edge for mounting the glass hook holders. The stirrer had a 1 inch by 2 inches paddle and rotated at 175 r.p.m. There were also holes in the lid to admit the tube from the reservoir, and an aerator. The tests were aerated continuously. These tests can be run for any length of time desired. Six coupons can be mounted in each test vessel. One was removed periodically to determine if the corrosion rates had leveled off. During the first few days of a test run the corrosion rates were relatively high and tended to be less reproducible, and for this reason it was necessary to run the test from 15-30 days. The initial corrosion rate for the system with no inhibitor present was about 80 m.p.y. After an exposure of 15 days, the rate will reach equilibrium at about 50 m.p.y.

*Test method C.*—These tests were designed as a modification of test method B, and have a heat transfer surface which would act as a specimen for evaluation of corrosion and fouling. The test unit had a reservoir, feed system, and test vessel identical to those of test method B, except that no oil bath was used. Solution was pumped from the vessel by means of a centrifugal pump, then vertically through the annular space between a 17 inch long,  $\frac{1}{2}$  inch out diameter (O.D.), 16 gauge tube, and

an outer glass jacket. The jacket was a 400 mm. West type condenser jacket. A  $\frac{3}{8}$  inch O.D. 500 watt heater, which was 16 inches long, was inserted inside of the tube. This tube acted as the test specimen, and was either a mild steel seamless tube, or an Admiralty metal tube.

After leaving the test heat exchanger, the solution flowed downwardly through a glass condenser, with cooling water in the jacket and back into the reservoir.

Rates of flow within this system are tabulated below:

10

|    | cc./sec. | $10^{-3}$ NRe | Velocity (ft./sec.) |
|----|----------|---------------|---------------------|
| 15 | 0        | 0             | 0                   |
|    | 53       | 25            | 1.4                 |
|    | 80       | 38            | 2.2                 |
|    | 97       | 46            | 2.6                 |
|    | 102      | 48            | 2.8                 |

20 The coding water flow to the jacket was controlled by means of a thermostat in the test vessel, so that the vessel could be maintained at any desired temperature which, in these tests, was either 95°, 125° or 160° F.

25 Using test method A, several of the quaternary ammonium salts in Table I were tested alone and in combination with sodium dichromate to determine their effectiveness. These results are presented below in Table II. The results were expressed in terms of P, F or G with the P indicating that the test material showed little or no activity, F meaning that it showed moderate activity, and G meaning that the material was good under the test conditions.

TABLE II

| 35 | Test No. | Description of test material                                                                | Evaluation         |                                      |
|----|----------|---------------------------------------------------------------------------------------------|--------------------|--------------------------------------|
|    |          |                                                                                             | Alone <sup>1</sup> | $\text{CrO}_4$ additive <sup>2</sup> |
| 40 | 1        | 2 - methyl - 1 - (2 - hydroxyethyl) - 1 - benzyl imidazolinium chloride.                    | P                  | G                                    |
|    | 2        | 2 - coco - 1 - (2 - hydroxyethyl) - 1 - benzyl imidazolinium chloride.                      | P                  | F                                    |
|    | 3        | 2 - coco - 1 - (hydroxyethyl) - 1 - (4 - chlorobutyl) imidazolinium chloride.               | F                  | G                                    |
|    | 4        | 2 - coco - 1 - (2 - hydroxyethyl) - 1 - octadecenyl imidazolinium chloride.                 | P                  | F                                    |
| 45 | 5        | 2 - tall oil fatty - 1 - (2 - hydroxyethyl) - 1 - benzyl imidazolinium chloride.            | F                  | G                                    |
|    | 6        | 2 - tall oil fatty - 1 - (2 - hydroxyethyl) - 1 - (4 - chlorobutyl) imidazolinium chloride. | P                  | G                                    |
|    | 7        | 2 - heptadecenyl - 1 - (2 - hydroxyethyl) - 1 - (4 - chlorobutyl) imidazolinium chloride.   | F                  | G                                    |
| 50 | 8        | 2 - heptadecyl - 1 - (2 - hydroxyethyl) - 1 - benzyl imidazolinium chloride.                | P                  | G                                    |
|    | 9        | 2 - heptadecyl - 1 - (hydroxyethyl) - 1 - octadecyl imidazolinium ethyl sulfate.            | P                  | G                                    |
|    | 10       | Dodecyl trimethyl ammonium chloride.                                                        | P                  | F                                    |
| 55 | 11       | Hexadecyl trimethyl ammonium chloride.                                                      | P                  | G                                    |
|    | 12       | Octadecyl trimethyl ammonium chloride.                                                      | P                  | G                                    |
|    | 13       | Coco trimethyl ammonium chloride.                                                           | P                  | G                                    |
|    | 14       | Soya trimethyl ammonium chloride.                                                           | P                  | G                                    |
|    | 15       | Tallow trimethyl ammonium chloride.                                                         | P                  | G                                    |
|    | 16       | Dieoco dimethyl ammonium chloride.                                                          | P                  | G                                    |
| 60 | 17       | Coco amine Rx 15 moles Eto quaternized with methyl chloride.                                | P                  | P                                    |
|    | 18       | Octadecyl amine Rx 2 moles Eto quaternized with methyl chloride.                            | P                  | G                                    |
|    | 19       | Octadecenyl amine Rx 2 moles Eto quaternized with methyl chloride.                          | P                  | G                                    |
| 65 | 19A      | Dihydrogenated tallow dimethyl ammonium chloride.                                           | P                  | P                                    |

70 <sup>1</sup> Using steel coupons, test material (200 p.p.m.) was evaluated as a corrosion inhibitor; pH 6.0-7.0; temperature 140° F.

<sup>2</sup> Using steel coupons, test material (40 p.p.m.) was evaluated as an additive to sodium dichromate (40 p.p.m.  $\text{CrO}_4$ ) to reduce corrosion and pitting; pH 6.0-7.0; temperature 140° F.

<sup>3</sup> Free from rosin acid components.

To further evaluate the invention, test method B was employed. The tests were designed to determine more critically conditions favoring the use of various ingredients. The treatment and test results are given in Table III.

TABLE III  
*Evaluation of Chromate-Zinc-Quaternary Treatments*  
 TREATMENT

| Test No. <sup>1</sup>                        | Composition No. from Table I | Continual, first week     |            |              | Remainder of run          |            |              | Quaternary in reservoir (5 days) |        | Analysis, p.p.m. in vessel, days |     |     |     |
|----------------------------------------------|------------------------------|---------------------------|------------|--------------|---------------------------|------------|--------------|----------------------------------|--------|----------------------------------|-----|-----|-----|
|                                              |                              | CrO <sub>4</sub> , p.p.m. | Zn, p.p.m. | Quat, p.p.m. | CrO <sub>4</sub> , p.p.m. | Zn, p.p.m. | Quat, p.p.m. | Theor.                           | Actual | 1                                | 8   | 22  | 28  |
| A. Effect of Quat Concentration              |                              |                           |            |              |                           |            |              |                                  |        |                                  |     |     |     |
| 1                                            | 12                           | 30                        | 2          | 2            | 30                        | 2          | 2            | 2                                | 2      |                                  |     |     |     |
| 2                                            | 12                           | 30                        | 2          | 5            | 30                        | 2          | 5            | 5                                | 5      |                                  |     |     |     |
| 3                                            | 12                           | 30                        | 2          | 40           | 30                        | 2          | 40           | 40                               | 40     |                                  |     |     |     |
| B. Effect of Zinc Concentration              |                              |                           |            |              |                           |            |              |                                  |        |                                  |     |     |     |
| 4                                            | 12                           | 30                        | 2          | 2            | 30                        | 2          | 2            | 2                                | 2      |                                  |     |     |     |
| 5                                            | 12                           | 30                        | 4          | 3            | 30                        | 4          | 3            | 3                                | 3      |                                  |     |     |     |
| 6                                            | 12                           | 30                        | 6          | 3            | 30                        | 6          | 3            | 3                                | 2.8    | 2.5                              | 0.7 | 0.4 | 1.0 |
| C. Effect of Initial Chromate Slug in Vessel |                              |                           |            |              |                           |            |              |                                  |        |                                  |     |     |     |
| 7                                            | 12                           | 20                        | 4          | 2            | 20                        | 4          | 2            | 2                                | 2.0    | 2.4                              | 1.9 | 0.6 | 1.0 |
| 8                                            | 12                           | 20                        | 4          | 2            | 20                        | 4          | 3            | 3                                | 1.9    | 1.3                              | 1.6 | 0.6 | 0.9 |
| 9                                            | 12                           | 20                        | 4          | 2            | 20                        | 4          | 2            | 2                                | 1.5    | 0.9                              | 1.0 | 0.9 |     |
| D. Effect of Treatment Level                 |                              |                           |            |              |                           |            |              |                                  |        |                                  |     |     |     |
| 10                                           | 12                           | 20                        | 4          | 2            | 30                        | 4          | 2            | 2                                | 2.0    | 1.0                              | 1.1 | 0.7 |     |
| 11                                           | 12                           | 30                        | 4          | 2            | 30                        | 4          | 2            | 2                                | 2.0    | 1.0                              | 1.1 | 0.7 | 0.8 |
| 12                                           | 12                           | 30                        | 6          | 3            | 30                        | 6          | 3            | 3                                | 2.8    | 2.5                              | 0.7 | 0.4 | 1.0 |
| 13                                           | 12                           | 30                        | 6          | 3            | 20                        | 4          | 2            | 2                                | 1.3    | 1.9                              | 2.3 | 1.9 | 2.1 |
| E. Comparison on Active Dosage Basis         |                              |                           |            |              |                           |            |              |                                  |        |                                  |     |     |     |
| 14                                           | 12                           | 30                        | 4          | 2            | 30                        | 4          | 2            | 2                                | 2.0    | 1.0                              | 1.1 | 0.7 | 0.8 |
| 15                                           | 19A                          | 30                        | 4          | 2            | 30                        | 4          | 2            | 2                                | 1.9    | 4.2                              | 0.8 | 0.8 | 0.4 |
| 16                                           | 8                            | 30                        | 4          | 2            | 30                        | 4          | 2            | 2                                | 0.5    | 1.3                              | 0.1 | 0.3 | 0.6 |
| F. Test without Quaternary                   |                              |                           |            |              |                           |            |              |                                  |        |                                  |     |     |     |
| 17                                           | Blank                        | 30                        | 2          |              | 30                        | 2          |              |                                  |        |                                  |     |     |     |

## OBSERVATIONS AND RESULTS

| Test No. <sup>1</sup>                        | Tuberculation-pitting evaluation, <sup>2</sup> days |   |   |    | Overall film formation | Cumulative corrosion, weight loss, mgs. |      |      |      | Overall corr. rate, m.p.y. |
|----------------------------------------------|-----------------------------------------------------|---|---|----|------------------------|-----------------------------------------|------|------|------|----------------------------|
|                                              | 1                                                   | 8 | 2 | 28 |                        | 1                                       | 8    | 22   | 28   |                            |
| A. Effect of Quat Concentration              |                                                     |   |   |    |                        |                                         |      |      |      |                            |
| 1                                            | 4                                                   | 3 | 2 | 2  | 4                      | 6.7                                     | 6.7  | 8.7  | 9.7  | 0.2                        |
| 2                                            | 4                                                   | 4 | 4 | 4  | 4                      | 3.0                                     | 5.9  | 7.6  | 7.1  | 0.2                        |
| 3                                            | 4                                                   | 4 | 3 |    | 4                      | 6.9                                     | 12.6 | 12.6 |      | 0.4                        |
| B. Effect of Zinc Concentration              |                                                     |   |   |    |                        |                                         |      |      |      |                            |
| 4                                            | 4                                                   | 3 | 2 | 2  | 4                      | 6.7                                     | 6.7  | 8.7  | 9.7  | 0.2                        |
| 5                                            | 4                                                   | 4 | 4 | 4  | 4                      | 3.0                                     | 3.5  | 6.6  | 7.3  | 0.2                        |
| 6                                            | 4                                                   | 4 | 4 | 4  | 4                      | 2.8                                     | 5.1  | 7.9  | 9.0  | 0.2                        |
| C. Effect of Initial Chromate Slug in Vessel |                                                     |   |   |    |                        |                                         |      |      |      |                            |
| 7                                            | 4                                                   | 3 | 3 | 2  | 4                      | 3.0                                     | 4.4  | 8.3  | 11.7 | 0.3                        |
| 8                                            | 4                                                   | 4 | 3 | 4  | 4                      | 2.0                                     | 3.3  | 6.8  | 8.7  | 0.2                        |
| 9                                            | 3                                                   | 3 | 3 |    | 4                      | 1.5                                     | 3.0  | 4.8  |      | 0.2                        |
| D. Effect of Treatment Level                 |                                                     |   |   |    |                        |                                         |      |      |      |                            |
| 10                                           | 2                                                   |   |   |    |                        | 8.6                                     |      |      |      |                            |
| 11                                           | 4                                                   | 4 | 4 | 4  | 4                      | 2.2                                     | 5.2  | 7.0  | 10.4 | 0.3                        |
| 12                                           | 4                                                   | 4 | 4 | 4  | 4                      | 2.8                                     | 5.1  | 7.9  | 9.0  | 0.2                        |
| 13                                           | 4                                                   | 4 | 4 | 4  | 4                      | 2.5                                     | 4.4  | 6.8  | 7.3  | 0.2                        |
| E. Comparison on Active Dosage Basis         |                                                     |   |   |    |                        |                                         |      |      |      |                            |
| 14                                           | 4                                                   | 4 | 4 | 4  | 4                      | 2.2                                     | 5.2  | 7.0  | 10.4 | 0.3                        |
| 15                                           | 4                                                   | 2 | 1 | 1  | 2                      | 2.6                                     | 5.8  | 9.0  | 10.6 | 0.3                        |
| 16                                           | 4                                                   | 2 | 1 | 1  | 2                      | 3.0                                     | 5.5  | 7.1  | 8.7  | 0.2                        |
| F. Test without Quaternary                   |                                                     |   |   |    |                        |                                         |      |      |      |                            |
| 17                                           | 2                                                   | 1 | 1 | 1  | 1                      | 34.6                                    | 58.1 | 71.0 |      | 22.7                       |

<sup>1</sup>All tests have an initial slug of 40 p.p.m., Composition 12, Table I.<sup>2</sup>Evaluation: 4—Excellent; 3—Good; 2—Unsatisfactory; 1—Poor.<sup>3</sup>22-day result.

To further evaluate the invention, test method C was employed in order to determine more completely the benefits of the inhibitors. These results are presented in Table IV.

sorption was only a small fraction of the rate of loss by normal blowdown. Thus, the loss of quaternary to the wood in a cooling tower would be a factor during the initial treatment but this is counteracted by increasing the

TABLE IV  
*Evaluation of Chromate-Zinc-Quaternary Treatments  
Obtained With Heat Transfer Apparatus*

| Pretreatment                                  |                          | Follow-up treatment          |            |                       |        |                   | Observations on tube |                             |               |
|-----------------------------------------------|--------------------------|------------------------------|------------|-----------------------|--------|-------------------|----------------------|-----------------------------|---------------|
| Type                                          | Quat. slug conc., p.p.m. | CrO <sub>4</sub> , p.p.m.    | Zn, p.p.m. | Quaternary (Table I)  |        | Test period, days | Film formation       | Grease removal              | Tuberculation |
|                                               |                          |                              |            | Type                  | p.p.m. |                   |                      |                             |               |
| A. Blank                                      |                          |                              |            |                       |        |                   |                      |                             |               |
| none.....                                     |                          | 40                           | 4          |                       |        | 14                |                      |                             | Heavy.        |
| B. Comparison of Quats on a Cost-Dosage Basis |                          |                              |            |                       |        |                   |                      |                             |               |
| Quat Slug <sup>1</sup> .....                  | 40                       | 30                           | 6          | 12                    | 3.0    | 8                 |                      |                             | Slight.       |
| Quat Slug <sup>1</sup> .....                  | 40                       | 30                           | 6          | 19A                   | 3.9    | 8                 |                      |                             | Do.           |
| Quat Slug <sup>1</sup> .....                  | 40                       | 30                           | 6          | 8                     | 6.0    | 8                 |                      |                             | Mod.          |
| C. Effect of Initial Quat Concentration       |                          |                              |            |                       |        |                   |                      |                             |               |
| Quat Slug <sup>1</sup> .....                  | 40                       | 30                           | 6          | 12                    | 5.0    | 12                |                      |                             | Slight.       |
| Quat Slug <sup>1</sup> .....                  | 60                       | 30                           | 6          | 12                    | 5.0    | 13                |                      |                             | Do.           |
| Quat Slug <sup>1</sup> .....                  | 80                       | 30                           | 6          | 12                    | 5.0    | 13                |                      |                             | Do.           |
| Quat Slug <sup>1</sup> .....                  | 60                       | 30                           | 6          | 12                    | 3.0    | 4                 |                      |                             | Mod.          |
| High Quat <sup>2</sup> .....                  | 60                       | 20                           | 4          | 12                    | 2.0    | 14                |                      |                             | Trace.        |
| Pretreatment                                  |                          | Quaternary in vessel, p.p.m. |            | Deposit analysis, mg. |        |                   |                      | Weight data                 |               |
| Type                                          | Quat. slug conc., p.p.m. | 3 day                        | 8 day      | PO <sub>4</sub>       | Ca     | Fe                | CR                   | Quat.                       | Zn            |
|                                               |                          |                              |            |                       |        |                   |                      | Scale+corr. prod.+film, mg. | Corr. loss    |
| A. Blank                                      |                          |                              |            |                       |        |                   |                      |                             |               |
| none.....                                     |                          |                              |            | 54                    | 155    |                   |                      | 503                         | 299           |
| B. Comparison of Quats on a Cost-Dosage Basis |                          |                              |            |                       |        |                   |                      |                             |               |
| Quat Slug <sup>1</sup> .....                  | 40                       | 1.2                          | 0.9        | 35                    | 49     | 2.3               | 22                   | 203                         | 86            |
| Quat Slug <sup>1</sup> .....                  | 40                       | 3.3                          | 0.4        | 35                    | 69     | 4.5               | 11                   | 243                         | 132           |
| Quat Slug <sup>1</sup> .....                  | 40                       | 2.1                          | 0.2        | 40                    | 96     | 1.3               | 15                   | 282                         | 140           |
| C. Effect of Initial Quat Concentration       |                          |                              |            |                       |        |                   |                      |                             |               |
| Quat Slug <sup>1</sup> .....                  | 40                       | 0.7                          | 0.9        | 96                    | 16     | 0.2               | 2.8                  | 308                         | 225           |
| Quat Slug <sup>1</sup> .....                  | 60                       | 1.6                          | 2.6        | 40                    | 15     | 2.5               | 15                   | 157                         | 81            |
| Quat Slug <sup>1</sup> .....                  | 80                       | 1.1                          | 1.5        | 50                    | 16     | 3.1               | 7                    | 174                         | 85            |
| Quat Slug <sup>1</sup> .....                  | 60                       | -----                        | -----      | 31                    | -----  | 0.3               | 6                    | 37                          | 42            |
| High Quat <sup>2</sup> .....                  | 60                       | 1.0                          | 1.0        | 22                    | 51     | 0                 | -----                | -----                       | 58            |

<sup>1</sup> Composition 12 of Table I used for slug in the test vessel at start of test.

<sup>2</sup> 30 p.p.m. CrO<sub>4</sub>, 6 p.p.m. Zn and 60 p.p.m. Comp. 12 for 4 days at 125° F.

To further illustrate the industrial utility of the invention, a typical quaternary ammonium compound, octadecyl trimethyl ammonium chloride was tested to determine its rate of absorption on redwood, a material commonly used in cooling tower construction. The test method may be briefly described as follows:

Extracted redwood blocks were placed in contact with a volume of the quaternary ammonium salt solution such that the area:volume ratio (34.5 sq. in.:1000 ml.) complied with the conditions of a typical cooling tower. In these tests the initial concentrations of the material were 20, 40, 80, and 120 p.p.m.; at intervals small samples (1% by volume) were withdrawn for analysis. The results (Table V) show that initially roughly 20 p.p.m. of the quaternary ammonium salt is absorbed but that the rate drops off after a few hours. Although the salt continued to be absorbed for the next three weeks, the rate of ab-

level of the initial high quaternary treatment. The results of these tests are presented in Table V below.

TABLE V  
*Absorption of Octadecyl Trimethyl Ammonium Chloride*

| Time (days) | Concentration of compound found (p.p.m.) |           |           |            |
|-------------|------------------------------------------|-----------|-----------|------------|
|             | 20 p.p.m.                                | 40 p.p.m. | 80 p.p.m. | 120 p.p.m. |
| 0           | 21                                       | 36        | 73        | 120        |
| 0.004       | 6                                        | 26        | 73        | 130        |
| 0.04        | 12                                       | 18        | 66        | 96         |
| 1           | 8                                        | 18        | 45        | 99         |
| 4           | 4                                        | 12        | 26        | 74         |
| 6           | 2                                        | 7         | 16        | 44         |
| 12          | 1.5                                      | 3         | 11        | 28         |
| 15          | 0.8                                      | 2         | 9         | 33         |
| 21          | 0.5                                      | 1         | 4         | 13         |

From Table II it will be observed that most of the quaternary ammonium salts tested were relatively inactive as inhibitors per se. When combined with the chromate, protection was afforded.

An interesting result presented in Table III is the fact that when the system was initially treated, using a high dosage of quaternary ammonium salt, e.g., 40 parts per million, and the lower concentration, viz., 5 parts per million was maintained, better protection was afforded than when the dosage of the quaternary ammonium salt was held constant throughout the test. The reason for this phenomenon is believed to be that the initial high dosage tends to form a protective coating on the surface which is subsequently maintained by the lower steady dosage.

Also observed from the results shown in Table III is that 40 parts per million of the quaternary ammonium salt, when maintained on a steady basis, is unnecessary once the protective coating is formed. The dosages from between 2 to 5 parts per million of the quaternary and from between 2 and 6 parts per million of the zinc salt give generally satisfactory results.

It becomes evident from the above tests that one method of practicing the invention is to feed relatively high dosages of the quaternary ammonium salts to the system to form an initial protective film which is then subsequently maintained by the use of lower continual dosages. The amount of quaternary ammonium salt used to form this protective film, as well as the time in which it takes the film to be formed, will, of course, be dependent upon the environmental factors present in each system. Thus, for instance, pH, temperature, dissolved solids, and the types of metals present must be taken into consideration. As a general rule, however, it may be stated that the protective films may be more readily formed by using large dosages of the quaternary ammonium salts for short periods of time rather than using smaller dosages for long periods of time. In the case of a typical cooling tower system at least 40 parts per million of the quaternary for at least 3 days should be used for forming the protective film.

The pretreatment with higher dosage quaternary ammonium salts provides a simple and effective method for stopping initial corrosion rates when industrial systems are first put on stream. It will be understood, however, that the invention does not require such a pretreatment operation since in most cases a continual feed of the chemical at low economical dosages will eventually form an effective protective film that will be self-maintaining.

As a further guide to forming an initial protective film of the quaternary ammonium salt, the pretreatment of the system should employ from 20 to 60 parts per million and preferably 30 to 40 parts per million of the quaternary salt for a period of time ranging from 7 hours to 30 days. Quite frequently only several days are required. The pretreatment is conducted using the same amount of chromate and heavy metal as previously specified.

In the specification, "EtO" is an abbreviation for ethylene oxide. Thus, in Table II, a test material coco amine Rx 15 moles EtO quaternized with methyl chloride refers to an amine derived from coconut oil which has been oxyalkylated with 15 moles of ethylene oxide per mole of amine and then reacted with one mole of methylene chloride per mole of amine.

The invention is hereby claimed as follows:

1. A non-corrosive industrial process water which comprises a major portion of water, at least 10 parts per million of a water soluble hexavalent compound of chromium, calculated as  $\text{CrO}_4$ , and at least 0.5 part per million of a water dispersible quaternary ammonium salt which contains at least one acyclic organic radical having at least 8 carbon atoms, the pH of said water being within the range of 5.5 to 8.5.

2. A non-corrosive industrial process water which comprises a major portion of water, 10 to 200 parts per million of a water soluble hexavalent compound of chromium, calculated as  $\text{CrO}_4$ , and 0.5 to 10 parts per million

of a water dispersible quaternary ammonium salt which has at least one acyclic organic radical of at least 12 carbon atoms in chain length, the pH of said water being within the range of 5.5 to 8.5.

3. A non-corrosive industrial process water which comprises a major portion of water, 10 to 200 parts per million of an alkali metal chromate, calculated as  $\text{CrO}_4$ , and 0.5 to 10 parts per million of a water dispersible quaternary ammonium halide which contains one acyclic organic radical of at least 16 carbon atoms in chain length, the pH of said water being within the range of 5.5 to 8.5.

4. A non-corrosive industrial process water which comprises a major portion of water, from 10 to 200 parts per million of an alkali metal chromate, calculated as  $\text{CrO}_4$ , and from 0.5 to 10 parts per million of a water dispersible quaternary ammonium chloride of the formula



where R is a higher aliphatic group of from 16 to 18 carbon atoms in chain length and  $\text{R}_1$ ,  $\text{R}_2$  and  $\text{R}_3$  are lower aliphatic hydrocarbon groups having from 1 to 6 carbon atoms, the pH of said water being within the range of 6.5 to 7.5.

5. The non-corrosive industrial process water of claim 4 where the water dispersible quaternary ammonium chromate is octadecyl trimethyl ammonium chloride.

6. A non-corrosive industrial process water which comprises a major portion of water, at least 10 parts per million of a water soluble hexavalent compound of chromium, calculated as  $\text{CrO}_4$ , at least 0.5 part per million of a water dispersible quaternary ammonium salt which contains at least 8 carbon atoms in an acyclic chain and at least 0.25 part per million of an ionizable compound having a cationic heavy metal radical from the group consisting of zinc, cobalt, nickel, mercury and trivalent chromium, the pH of said water being within the range of 5.5 to 8.5.

7. A non-corrosive industrial process water which comprises a major portion of water, at least 10 parts per million of a water soluble hexavalent compound of chromium, calculated as  $\text{CrO}_4$ , at least 0.5 part per million of a water dispersible quaternary ammonium salt which has at least one acyclic organic radical of at least 12 carbon atoms in chain length, and at least 0.25 part per million of an ionizable compound having a cationic heavy metal radical from the group consisting of zinc, cobalt, nickel, mercury and trivalent chromium, the pH of said water being within the range of 5.5 to 8.5.

8. A non-corrosive industrial process water which comprises a major portion of water, at least 10 parts per million of an alkali metal chromate, calculated as  $\text{CrO}_4$ , at least 0.5 part per million of a water dispersible quaternary ammonium halide which contains one acyclic organic radical of at least 16 carbon atoms in chain length and from 0.25 to 6 parts per million of an ionizable compound having a cationic heavy metal radical from the group consisting of zinc, cobalt, nickel, mercury and trivalent chromium, the pH of said water being within the range of 5.5 to 8.5.

9. A non-corrosive industrial process water which comprises a major portion of water, from 10 to 200 parts per million of an alkali metal chromate, calculated as  $\text{CrO}_4$ , from 0.5 to 10 parts per million of a water dispersible quaternary ammonium chloride of the formula



where R is a higher aliphatic group of from 16 to 18 carbon atoms in chain length and  $\text{R}_1$ ,  $\text{R}_2$  and  $\text{R}_3$  are lower aliphatic hydrocarbon groups having from 2 to 6 carbon atoms, and from 2 to 6 parts per million of an ionizable compound having a cationic heavy metal radical from the group consisting of zinc, cobalt, nickel, mercury and tri-

valent chromium, the pH of said water being within the range of from 6.5 to 7.5.

10. The non-corrosive industrial process water of claim 9 wherein the water dispersible quaternary ammonium chloride is octadecyl trimethyl ammonium chloride and the ionizable compound of the heavy metal has a cationic zinc radical.

11. The non-corrosive industrial process water of claim 9 which also contains from 0.5 to 2 parts per million of a molecularly dehydrated phosphate, calculated as  $\text{PO}_4$ .

12. The process of protecting metals against corrosion by contact with aqueous liquids which comprises feeding from separate supply sources into an aqueous industrial process water having a pH within the range of 5.5 to 8.5, an amount of a water soluble hexavalent compound of chromium calculated as  $\text{CrO}_4$  sufficient to provide in said water at least 10 parts per million thereof, and an amount of a water dispersible quaternary ammonium salt sufficient to provide from 20 to 60 parts per million thereof in said water, said quaternary ammonium salt having at least one acyclic organic radical with at least 8 carbon atoms, contacting the metals of an aqueous process system with said water subsequent to said feeding, for a period of time ranging from 7 hours to 30 days sufficient to establish a protective film on said metals, and then continuing to treat said metals with said water while maintaining feeding of said quaternary salt in amounts sufficient to maintain said protective film.

13. The process of claim 12 wherein feeding is sufficient to provide in said water from 10 to 200 parts per million of a water soluble hexavalent compound of chromium, and 0.5 to 10 parts per million of a water dispersible quaternary ammonium salt, and wherein the said quaternary ammonium salt has at least one acyclic organic radical of at least 12 carbon atoms in chain length.

14. The process of claim 13 wherein the water soluble hexavalent compound of chromium is an alkali metal chromate and the water dispersible quaternary ammonium salt is a quaternary ammonium halide having one acyclic organic radical of at least 16 carbon atoms in chain length.

15. The process of claim 14 wherein the quaternary ammonium halide has the formula:



where R is a higher aliphatic group of from 16 to 18 carbon atoms in chain length and R<sub>1</sub>, R<sub>2</sub> and R<sub>3</sub> are lower aliphatic hydrocarbon groups having from 1 to 6 carbon atoms.

16. The process of claim 15 wherein the quaternary ammonium halide is octadecyl trimethyl ammonium chloride.

17. The process of protecting metals against corrosion by contact with aqueous liquids which comprises feeding from separate supply sources into an aqueous industrial process water having a pH within the range of 5.5 to 8.5, an amount of a water soluble hexavalent compound of chromium calculated as  $\text{CrO}_4$  sufficient to provide in said water at least 10 parts per million thereof, and an amount

of a water dispersible quaternary ammonium salt sufficient to provide from 20 to 60 parts per million thereof in said water, and also feeding into said water from a supply source in an amount sufficient to provide in said water at least 0.25 part per million of an ionizable compound having a cationic heavy metal radical from the group consisting of zinc, cobalt, nickel, mercury and trivalent chromium, said quaternary ammonium salt having at least one acyclic organic radical with at least 8 carbon atoms, contacting the metals of an aqueous process system with said water subsequent to said feeding for a period of time ranging from 7 hours to 30 days sufficient to establish a protective film on said metals, and then continuing to treat said metals with said water while maintaining feeding of said quaternary salt in amounts sufficient to maintain said protective film.

18. The process of claim 17 wherein the quaternary ammonium salt has at least one acyclic organic radical of at least 12 carbon atoms in chain length.

19. The process of claim 18 wherein the quaternary ammonium salt is a quaternary ammonium halide containing one acyclic organic radical of at least 16 carbon atoms in chain length, and wherein feeding is sufficient to provide in said water from 0.25 to 6 parts per million of said ionizable compound having a cationic heavy metal radical.

20. The process of claim 19 wherein the quaternary ammonium halide has the formula:



where R is a higher aliphatic group of from 16 to 18 carbon atoms in chain length and R<sub>1</sub>, R<sub>2</sub> and R<sub>3</sub> are lower aliphatic hydrocarbon groups having from 1 to 6 carbon atoms, and wherein feeding is sufficient to provide in said water 2 to 6 parts per million of said ionizable compound having a cationic heavy metal radical, and wherein the pH of said water is within the range of from 6.5 to 7.5.

21. The process of claim 20 wherein the quaternary ammonium chloride is octadecyl trimethyl ammonium chloride and the ionizable compound of a heavy metal has a cationic zinc radical.

22. The process of claim 21 wherein feeding is further maintained sufficient to provide in said water from 0.5 to 2 parts per million of a molecularly dehydrated phosphate, calculated as  $\text{PO}_4$ .

#### References Cited in the file of this patent

#### UNITED STATES PATENTS

|           |               |               |
|-----------|---------------|---------------|
| 2,274,058 | Goebel et al. | Feb. 24, 1942 |
| 2,325,359 | Arnold et al. | July 27, 1943 |
| 2,711,391 | Kahler        | June 21, 1955 |
| 2,738,325 | Rydell        | Mar. 13, 1956 |
| 2,793,932 | Kahler et al. | May 28, 1957  |
| 2,872,281 | Kahler et al. | Feb. 3, 1959  |
| 2,877,085 | George et al. | Mar. 10, 1959 |
| 2,900,222 | Kahler et al. | Aug. 18, 1959 |
| 2,947,703 | Larsonneur    | Aug. 2, 1960  |

UNITED STATES PATENT OFFICE  
CERTIFICATE OF CORRECTION

Patent No. 3,079,220

February 26, 1963

David B. Boies et al.

It is hereby certified that error appears in the above numbered patent requiring correction and that the said Letters Patent should read as corrected below.

Column 12, line 72, for "2" read -- 1 --.

Signed and sealed this 17th day of December 1963.

(SEAL)

Attest:

ERNEST W. SWIDER

Attesting Officer

EDWIN L. REYNOLDS

Acting Commissioner of Patents